

# United States Patent Office

2,927,691

Patented Mar. 8, 1960

1

2,927,691

## PROCESS OF DEOILING PHOSPHATE CONCENTRATE BY MEANS OF IMMISCIBLE LIQUIDS

Otto Charles Chapman, Lakeland, and Arnold Walker Dean, Nichols, Fla., assignors to Virginia-Carolina Chemical Corporation, Richmond, Va., a corporation of Virginia

No Drawing. Application December 30, 1954  
Serial No. 478,918

7 Claims. (Cl. 209—166)

The present invention is concerned with the concentration of phosphate minerals from their ores of the type found in the Florida pebble phosphate field and more especially with an improved double flotation process. Specifically our invention embodies an improved process for deoiling the rougher phosphate concentrate produced in the first step of the double float process.

Phosphate flotation methods were, for many years, confined to the use of anionic collecting agents with the resultant flotation of a phosphate bearing froth which contained silica to the extent of about 6%. With the advent of U.S. Patents 2,222,728 and 2,293,640, issued respectively to Francis X. Tartaron and Arthur Crago, the phosphate industry switched almost exclusively to the use of a combination of anionic and cationic reagents. In this combination the phosphate feed is first oiled with a fatty acid (anionic) reagent, in order to float a silica bearing phosphate froth. This is followed by a deoiling step to remove the effect of the anionic reagent and finally by a recoating with a cationic reagent and flotation to produce a low-silica, phosphate machine discharge product. This is the essence of the so-called double flotation process.

According to the double flotation method now practiced extensively in the industry, the phosphate ore of about minus 35-mesh, relatively free of slime and containing about 70% solids is conditioned with a negative-ion (anionic) agent and fed to the flotation cells. The negative-ion agent collects and removes a rougher concentrate containing a high proportion of the phosphate values mixed with some silicious gangue. This first concentration step can be carried out in such a manner as to collect almost the whole amount of the phosphate present in the ore but the rougher concentrate so obtained will still contain from 10 to 20% of silica.

Examples of negative-ion agents which may be used in carrying out the first concentrating operation have been listed in U.S. 2,293,640 and comprise the higher fatty acids, such as fish oil fatty acid and oleic acid and their soaps. They include the resin acids and their soaps, wood by-product fatty acids, naphthenic acids and their salts, the higher sulfo-fatty acids and their salts formed from appropriate bases, acid esters of high-molecular-weight aliphatic alcohols with inorganic acids and their salts and high molecular weight xanthates and other similar compounds.

In present practice the rougher phosphate concentrate is deoiled with a mineral acid, as for example according to U.S. 2,293,640. It has been the general belief that it is necessary to remove completely the anionic, fatty acid reagent before carrying out the cationic amine flotation step. Since the fatty acids are normally oils, this step has become known as a deoiling process. U.S. 2,599,530 suggests that if a small amount of mineral acid is allowed to remain on the rougher concentrate that the silica will be activated and more easily floated in the succeeding cationic concentration step.

It is a prime object of our invention to dispense entirely with the use of mineral acids for deoiling the

2

rougher concentrate. Corrosion is a very big problem in the flotation industry and a large amount of this corrosion can be attributed to the dilute acids employed in this deoiling step. To eliminate the use of these acids and thereby to eliminate the need for handling acids in the flotation operation would materially aid in the control of corrosion. This deoiling treatment is the only step in the entire phosphate flotation process where strong mineral acids are employed. Their elimination here would thus remove them from the complete process. It is an object of our invention to deoil the rougher concentrate by a process which does not employ corrosive or hazardous materials.

An additional and equally important object is to provide a process for deoiling which will be superior to those processes now practiced and one which will leave the surface of the silica, contained admixed with phosphate in the rougher phosphate concentrate, in such a state that it is more readily floated in the succeeding cationic, amine flotation.

Before describing the actual process of our invention it is necessary to very briefly outline the succeeding cationic, amine flotation process. Any true tests of the amount of deoiling must include the subsequent amine flotation with analyses of the resultant fractions.

The deoiled, rougher phosphate concentrate is returned to the flotation machine where it is formed with water into a dilute pulp of about 25% solids and, without preliminary agitation, frothed for one minute or longer in the presence of a cationic amine reagent and kerosene. The almost pure silica is floated and is removed by the scrapers. The material which remains in the machine constitutes the finished phosphate concentrate. Examples of cationic amine reagents which may be used in carrying out this second flotation step are the higher aliphatic amines and their salts with water-soluble acids, the esters of amino-alcohols with high molecular weight fatty acids and their salts with water-soluble acids, the resin amines and their salts with water-soluble acids and the higher aliphatic 30 quaternary ammonium bases, including pyridine, quinoline and other heterocyclics capable of forming quaternary compounds, and their salts with water-soluble acids. These various examples are not, of course, equally effective or useful in this process. The use of a cationic active 35 amine or an amine salt generally is preferred. As will be 40 illustrated, the actual reagent used in the tests of our invention is a mixture of two amine salts.

The above and other objects are accomplished by the practice of our invention. We have discovered that excellent deoiling is obtained by the use of water-immiscible 45 organic solvents, among which the organic esters of carboxylic acids give best results. By water-immiscible organic solvents we refer to those organic liquids which are substantially insoluble in water (solubility of about 55 less than 5% at room temperature) and which do not possess substantial vapor pressure at room temperature or vapor pressure which would make them either a health or a fire hazard. We have discovered that the addition of such immiscible organic solvents in the deoiling step 60 results in excellent deoiling and eliminates or takes the place of the use of the corrosive and hazardous mineral acid. Furthermore the use of these liquids as deoilers appears to prepare the surface of the silica so that it is more amenable to flotation in the succeeding cationic 65 flotation. This is an unusual and entirely unpredictable result. As will be illustrated, these organic liquids are used at a concentration of about 0.5% which is a very small amount when the large amounts of water slurries of phosphate handled in the flotation procedures are considered. Certainly our process does not embody an organic solvent extraction in the sense that such extractions

are practiced in the organic chemicals industry where large volumes of solvents are used to dissolve and extract small amounts of other materials. The small amounts of immiscible organic solvents which we employ appear to aggregate the oily fatty acid in droplets or globules in such a manner that the rougher concentrate is effectively deoiled, the oil being removed from the mixture in the water washing after the treatment with the organic liquids. Our deoiling agents are referred to as solvents because, although as noted above, their use is not a solvent extraction of the anionic reagent in the usual sense, they are solvents of the anionic reagents.

The residual effects of these liquids on the phosphate and silica can not be entirely explained. Certainly it is an unusual one and one which was entirely unexpected. It is difficult to see how these organic liquids can "activate" the surface of the inorganic silica in the sense referred to in U.S. Patent 2,599,530. It is equally difficult to fit these liquids into the theory that silica floats in the cationic flotation step because of the formation of hydrated silicic acid on the surface of the silica particles. We offer as a possible explanation of the resultant excellent flotation of silica the fact that very small amounts of the organic liquids which remain on the silica and phosphate act as frothers themselves or these liquids, which are normally commercial products, may contain even smaller amounts of unesterified organic alcohols which are known frothers. This would result in a better froth and could conceivably result in a better flotation separation. Our invention is not limited to any of the suggested explanations as to how and why these immiscible organic solvents function. We have discovered a new and novel method for deoiling the rougher phosphate concentrate employing immiscible organic solvents and this process results in a superior froth flotation in the succeeding cationic separation.

Immiscible organic solvents which we have found to be operable in the practice of our invention include normally liquid aliphatic hydrocarbons as included in petroleum oils, terpene hydrocarbons and their derivatives, normally liquid halogenated hydrocarbons, and esters. Water-immiscible liquids which possess low vapor pressures and are not hazardous and which do not contain hydrolysable or water-reactive groupings generally are operable. Such compounds include, aromatic hydrocarbons of higher molecular weight, higher molecular weight alcohols, aldehydes, glycols and glycol derivatives, ketones, ethers or higher molecular weight, acetals, nitrogen derivatives, sulfur derivatives and mixtures of these and other groupings.

Having described our invention in general terms we will illustrate the process with specific examples which include samples of organic liquid from the many chemical groupings listed above.

All samples used in the illustrative examples of this invention were taken from the rougher concentrate produced in the No. 91 Flotation Plant of Virginia-Carolina Chemical Corporation, Bartow, Florida. The rougher concentrate from this plant is at least about 90% minus 35-mesh and contains about 80% solids.

To produce this rougher concentrate, phosphate debris, which contains phosphate rock and silica and runs roughly minus 14-mesh in size, is hydraulically classified in

order to separate the minus 35-mesh fraction. The minus 35-mesh product is dewatered and deslimed in a rake classifier. The discharge, which runs approximately 70% solids, is fed to a conditioner where 0.6 lbs./ton of caustic soda, 3 lbs./ton of Bunker C-No. 2 fuel oil (resultant specific gravity 18-20° API), and 0.7 lb./ton of tall oil are added, with agitation. Conditioning time is two minutes. The discharge is diluted with about 4 parts of water to each part of discharge and the mixture is fed to the flotation cells. The froth product from these cells is known as the rougher concentrate and contains a high percentage of phosphate but also some silica.

1270 gram-samples (1000 g., dry weight) of this rougher concentrate were placed in a beaker and the deoiling agent to be evaluated was added and the resultant mixture was stirred for three minutes. The thus deoiled mixture was washed by decantation until a relatively clear wash water was obtained. Normally 12 to 16 liters of water was required for this washing. The washed solid material was placed in a Fagergren laboratory flotation machine and water was added to the top of the conical part of the test-bowl. This corresponds to a dilution of approximately 2-3 parts of water to 1 part of solids. The cationic amine reagent and kerosene were added and the mixture was agitated without frothing for about 15 secs. In all tests the cationic amine reagent was a mixture composed of 50% rosin amine D acetate, a product of the Hercules Powder Co., and 50% Armac T, produced by Armour & Co. Armac T comprises the acetate salts of a mixture of 30% hexadecyl, 25% octadecyl and 45% octadecenyl amines. After the 15-second agitation the flotation machine was filled with water. Air was admitted to begin frothing and the thus formed matter-froth float was carefully removed, normally with a flexible rubber scraper.

Table I is a summary of the results of deoiling rougher phosphate concentrate with immiscible organic solvents. Test No. 1 has been included to illustrate the results obtained with present deoiling practices which employ sulfuric acid, as for example in U.S. Patent 2,293,640. The percent of BPL recovery in the froth fraction is inversely proportional to the effectiveness of the deoiling. The most efficient or effective deoiling compounds will give the lowest grade froth product. Phosphate which has not been deoiled will, of course, float with the silica in the cationic floatation step. A low percentage of insoluble matter in the concentrate, expressed as "percent Insol." in Table I is also desirable but is not quite as accurate an evaluation of deoiling as is a low percent BPL recovery in the froth. The percent insol. should be kept in mind as it is a measure of unfloated silica which remains in the final phosphate concentrate. Both low BPL in the froth and low insol. in the concentrate are desirable.

The deoiling agents may be added as such or in admixture with water.

In the following table all weights refer to dry weights. The mixture of ore and deoiler must be sufficiently fluid to be stirrable, the upper limit of solids content being about 80%. If more dilute mixtures are used the stirring of the mixture must be prolonged.

In the table the last column headed "Deoiled at —% solids" refers to the solids content of the mixture of ore, deoiler and water.

Table I

| Test No. | Product | Percent Weight | Percent BPL | Percent Insol. | Percent BPL Recovered | Deoiling and cationic agents   | Lbs. per Ton of Feed | Deoiled at — Percent Solids |
|----------|---------|----------------|-------------|----------------|-----------------------|--------------------------------|----------------------|-----------------------------|
| 1        | Feed    | 100.0          | 60.0        |                | 100.0                 | H <sub>2</sub> SO <sub>4</sub> | 6.00                 |                             |
|          | Froth   | 25.7           | 16.4        |                | 7.0                   | Kerosene                       | 1.00                 | 50                          |
|          | Conc.   | 74.3           | 75.1        | 6.9            | 93.0                  | Amine                          | 0.22                 |                             |
|          | Feed    | 100.0          | 60.2        |                | 100.0                 | Diesel oil                     | 9.50                 |                             |
| 2        | Froth   | 27.2           | 12.3        |                | 5.6                   | Kerosene                       | 1.00                 | 75                          |
|          | Conc.   | 72.8           | 78.1        | 3.7            | 94.4                  | Amine                          | 0.20                 |                             |

See footnotes at end of table.

Table I—Continued

| Test No. | Product | Percent Weight | Percent BPL | Percent Insol. | Percent BPL Recovered | Deoiling and cationic agents | Lbs. per Ton of Feed | Deoiled at—Percent Solids |
|----------|---------|----------------|-------------|----------------|-----------------------|------------------------------|----------------------|---------------------------|
| 3        | Feed    | 100.0          | 70.4        |                | 100.0                 | Diesel oil                   | 10.00                |                           |
|          | Froth   | 15.7           | 12.1        |                | 2.7                   | Kerosene                     | 0.75                 | 75                        |
|          | Conc.   | 84.3           | 81.3        | 2.5            | 97.3                  | Amine                        | 0.21                 |                           |
| 4        | Feed    | 100.0          | 71.0        |                | 100.0                 | "Yarmour F" Pine oil         | 10.5                 |                           |
|          | Froth   | 9.5            | 27.3        |                | 3.7                   | Kerosene                     | 0.5                  | 75                        |
|          | Conc.   | 90.5           | 75.6        | 2.2            | 96.3                  | Amine                        | 0.22                 |                           |
| 5        | Feed    | 100.0          | 71.2        |                | 100.0                 | "Frother B 23"               | 9.4                  |                           |
|          | Froth   | 10.7           | 32.5        |                | 4.9                   | Kerosene                     | 0.5                  | 76                        |
|          | Conc.   | 89.3           | 75.8        | 2.2            | 95.1                  | Amine                        | 0.22                 |                           |
| 6        | Feed    | 100.0          | 62.0        |                | 100.0                 | Chloroform                   | 16.50                |                           |
|          | Froth   | 26.9           | 16.1        |                | 7.0                   | Kerosene                     | 1.00                 | 75                        |
|          | Conc.   | 73.1           | 78.9        | 3.5            | 93.0                  | Amine                        | 0.20                 |                           |
| 7        | Feed    | 100.0          | 62.2        |                | 100.0                 | Carbon tetrachloride         | 17.70                |                           |
|          | Froth   | 24.4           | 9.7         |                | 3.8                   | Kerosene                     | 1.00                 | 75                        |
|          | Conc.   | 75.6           | 79.1        | 3.3            | 96.2                  | Amine                        | 0.20                 |                           |
|          | Feed    | 100.0          | 61.8        |                | 100.0                 | Crude sulphate turpentine    | 9.50                 |                           |
| 8        | Froth   | 34.2           | 28.9        |                | 16.0                  | Kerosene                     | 1.00                 | 75                        |
|          | Conc.   | 65.8           | 78.9        | 3.6            | 84.0                  | Amine                        | 0.20                 |                           |
|          | Feed    | 100.0          | 62.1        |                | 100.0                 | Alpha pinene                 | 9.50                 |                           |
| 9        | Froth   | 31.3           | 24.3        |                | 12.2                  | Kerosene                     | 1.00                 | 75                        |
|          | Conc.   | 68.7           | 79.3        | 3.2            | 87.8                  | Amine                        | 0.20                 |                           |
| 10       | Feed    | 100.0          | 70.7        |                | 100.0                 | Butyl acetate                | 10.00                |                           |
|          | Froth   | 12.5           | 6.6         |                | 1.2                   | Kerosene                     | 0.75                 | 75                        |
|          | Conc.   | 87.5           | 79.9        | 4.5            | 98.8                  | Amine                        | 0.21                 |                           |
|          | Feed    | 100.0          | 70.2        |                | 100.0                 | 2-ethylhexyl acetate         | 10.00                |                           |
| 11       | Froth   | 13.6           | 6.8         |                | 1.3                   | Kerosene                     | 0.75                 | 75                        |
|          | Conc.   | 86.4           | 80.2        | 3.5            | 98.7                  | Amine                        | 0.21                 |                           |
|          | Feed    | 100.0          | 61.9        |                | 100.0                 | Octyl acetate                | 9.90                 |                           |
| 12       | Froth   | 24.2           | 7.7         |                | 3.0                   | Kerosene                     | 1.00                 | 75                        |
|          | Conc.   | 75.8           | 79.2        | 2.8            | 97.0                  | Amine                        | 0.20                 |                           |
|          | Feed    | 100.0          | 70.1        |                | 100.0                 | Diethyl carbonate            | 10.00                |                           |
| 13       | Froth   | 13.6           | 8.0         |                | 1.5                   | Kerosene                     | 0.75                 | 75                        |
|          | Conc.   | 86.4           | 79.9        | 3.7            | 98.5                  | Amine                        | 0.21                 |                           |
|          | Feed    | 100.0          | 70.6        |                | 100.0                 | Diethyl phthalate            | 10.00                |                           |
| 14       | Froth   | 13.0           | 7.5         |                | 1.4                   | Kerosene                     | 0.75                 | 75                        |
|          | Conc.   | 87.0           | 80.0        | 4.2            | 98.6                  | Amine                        | 0.21                 |                           |
|          | Feed    | 100.0          | 70.4        |                | 100.0                 | 2-ethylhexyl phthalate       | 10.00                |                           |
| 15       | Froth   | 14.9           | 10.6        |                | 2.2                   | Kerosene                     | 0.75                 | 75                        |
|          | Conc.   | 85.1           | 80.9        | 2.9            | 97.8                  | Amine                        | 0.21                 |                           |
|          | Feed    | 100.0          | 70.2        |                | 100.0                 | Diethyl adipate              | 100.0                |                           |
| 16       | Froth   | 14.8           | 10.2        |                | 2.1                   | Kerosene                     | 0.75                 | 75                        |
|          | Conc.   | 85.2           | 80.6        | 2.9            | 97.9                  | Amine                        | 0.21                 |                           |
|          | Feed    | 100.0          | 70.2        |                | 100.0                 | Butyl stearate               | 10.00                |                           |
| 17       | Froth   | 16.3           | 14.5        |                | 3.4                   | Kerosene                     | 0.75                 | 75                        |
|          | Conc.   | 83.7           | 81.1        | 2.4            | 96.6                  | Amine                        | 0.21                 |                           |
|          | Feed    | 100.0          | 70.3        |                | 100.0                 | n-Hexyl furoate              | 10.00                |                           |
| 18       | Froth   | 14.8           | 9.0         |                | 1.9                   | Kerosene                     | 0.75                 | 75                        |
|          | Conc.   | 85.2           | 80.9        | 2.6            | 98.1                  | Amine                        | 0.21                 |                           |
|          | Feed    | 100.0          | 70.3        |                | 100.0                 | Foilene                      | 10.00                |                           |
| 19       | Froth   | 24.3           | 35.9        |                | 12.4                  | Kerosene                     | 0.75                 | 75                        |
|          | Conc.   | 75.7           | 81.3        | 2.1            | 87.6                  | Amine                        | 0.21                 |                           |

## NOTES TO TABLE I

Test 4.—Yarmour "F" Pine Oil is a product of Hercules Powder Company. It is produced by the solvent extraction of southern pine stump wood and consists largely of terpene alcohols. Composition varies but it is normally 70 to 80% of a mixture of the tertiary and secondary terpene alcohols—alpha terpineol, borneol, and fenchyl alcohol. The balance is composed mainly of the hydrocarbon—dipentene, with minor amounts of the ketones—fenchone and camphor—and the ethers—anethole and estragole.

Test 5.—Frother B23 is a product marketed by E. I. du Pont de Nemours & Co. and consists of 40-45% of 2,4-dimethylpentanol, 40-45% of 2,4-dimethylhexanol and 8-10% of unidentified ketones.

Test 19.—Foilene is an ester obtained from cottonseed oil.

It can be readily seen that substantially all of these immiscible organic solvents are at least equal, and most of them are superior, to the sulfuric acid of present practice. They yield froth products which contain a lower percent of BPL than the froth obtained after deoiling with sulfuric acid and their percent insol. in the concentrate is as low or less than that which remains after sulfuric acid treatment. The deoiling obtained with the organic esters, tests 10-18, is particularly outstanding as shown by the very low percent BPL recoveries in the froth products.

Tests 2 and 3 which employed diesel oil as a deoiler are also important from an economic standpoint since diesel oil sells for only a few cents a pound. This deoiling process can compete cost-wise with even the mildest sulfuric acid deoiling of present practice. It is also noted that the other organic solvents disclosed as deoilers are all commercially available in quantities and price ranges which would render them competitive when the higher grade products which they yield are considered. Also the organic liquids illustrated are non-hazardous, easily handled and thoroughly eliminate the necessity of handling corrosive mineral acids.

It will be understood from the foregoing disclosure that our invention is not concerned with the anionic and

cationic flotation agents used in the two flotation steps which precede and follow the deoiling step, such agents being well known in the art.

The quantity of the deoiling agent to be used is generally within the range from about 5 to about 25 pounds per ton of ore treated. As shown by the tests, about 10 pounds per ton generally gives good results. The quantity to be used in any particular instance may of course readily be determined by a series of tests. As little as 3 pounds of diesel oil has been used effectively.

The deoiling agent conveniently and effectively is applied as disclosed above by stirring it with the wet ore, i.e. a mixture of ore and water containing about 75 to 80% by weight of ore, but the agent may be applied by stirring it with the dry ore or with ore-water mixtures containing higher ratios of water.

The pH of the ore-water mixtures have been observed and have not been found to exert an appreciable effect. It may be said that a pH within the range from 7 to 8 gives satisfactory results.

We claim:

1. In a process for the beneficiation of phosphate ore containing siliceous impurities involving the steps in sequence of anionic flotation, deoiling the resulting concentrate and cationic flotation of the deoiled concentrate,

the improvement which consists in deoiling the concentrate produced by the anionic flotation by mixing the concentrate containing not more than about 80% of solids and at least about 20% of water in the absence of a water-soluble strong mineral acid with from about 3 to about 25 pounds per ton of solids of a normally liquid organic solvent which is immiscible and non-reactive with water selected from the group consisting of diesel oil, a product containing from 70% to 80% of a mixture of secondary and tertiary terpene alcohols, a product containing 40-45% of 2,4-dimethylpentanol and 40-45% of 2,4-dimethylhexanol, chloroform, carbon tetrachloride, crude sulfate turpentine, alpha pinene, the alkyl esters of mono- and dicarboxylic acids the alkyl groups of which contain from 2 to 8 carbon atoms, diethyl carbonate, hexyl furoate and an ester of cotton seed oil.

2. Process as defined in claim 1 in which a mixture of about 2000 parts by weight of ore concentrate with about 600 parts by weight of water is mixed with about 10 parts by weight of the solvent.

3. Process as defined in claim 1 in which the organic solvent is diesel oil.

4. Process as defined in claim 1 in which the organic

solvent is a product containing from 70% to 80% of a mixture of secondary and tertiary terpene alcohols.

5. Process as defined in claim 1 in which the organic solvent is a product containing 40-45% of 2,4-dimethylpentanol and 40-45% of 2,4-dimethylhexanol.

6. Process as defined in claim 1 in which the organic solvent is an alkyl ester of acetic acid the alkyl group of which contains from 2 to 8 carbon atoms.

7. Process as defined in claim 1 in which the organic solvent is an alkyl ester of phthalic acid the alkyl group of which contains from 2 to 8 carbon atoms.

References Cited in the file of this patent

UNITED STATES PATENTS

|    |           |             |       |                |
|----|-----------|-------------|-------|----------------|
| 15 | 1,312,266 | Navin       | ----- | Aug. 5, 1919   |
|    | 1,615,121 | Flyeman     | ----- | Jan. 18, 1927  |
|    | 2,173,842 | Horner      | ----- | Sept. 26, 1939 |
|    | 2,293,640 | Crago       | ----- | Aug. 18, 1942  |
| 20 | 2,461,813 | Duke        | ----- | Feb. 15, 1949  |
|    | 2,524,859 | Van Dongen  | ----- | Oct. 10, 1950  |
|    | 2,753,997 | Duke et al. | ----- | July 10, 1956  |